

(No Model.)

F. DE LALANDE & G. CHAPERON.

GALVANIC BATTERY.

No. 274,110.

Patented Mar. 20, 1883.



Witnesses.

C. E. Lusby

Prof. W. Hay

Inventors

Felix de Lalande,  
and  
Georges Chaperon.

By  
John J. Halsted & Son,  
their Atts.,

# UNITED STATES PATENT OFFICE.

FELIX DE LALANDE, OF PARIS, FRANCE, AND GEORGES CHAPERON, OF MINES D'ALOSNO, SPAIN.

## GALVANIC BATTERY.

SPECIFICATION forming part of Letters Patent No. 274,110, dated March 20, 1883.

Application filed July 11, 1882. (No model.) Patented in France June 25, 1881, No. 143,644.

*To all whom it may concern:*

Be it known that we, FELIX DE LALANDE and GEORGES CHAPERON, citizens of the Republic of France, residing respectively at Paris, in the Republic of France, and the Mines d'Alonso, Province de Huelva, in the Kingdom of Spain, have jointly invented certain new and useful Improvements in Galvanic Batteries, for which we have received Letters Patent or Brevet d'Invention in France No. 143,644, dated 25th June, 1881; and we do hereby declare that the following is a full, clear, and exact description of the invention, which will enable others skilled in the art to which it app pertains to make and use the same.

These piles are characterized by the employment simultaneously of oxide of copper as the depolarizing-body and of caustic potash or caustic soda in solution as the exciting-liquid. They can be readily formed with oxide-of-copper electrodes of good depolarizing-power having a good conductivity, especially when they already have worked and contain some metallic copper. We employ these caustic solutions in place of other solutions because we have found that they possess very good conductivity and that the oxide of copper is insoluble therein. Other solutions we have as the result of experiment not found to possess these two advantages at once. The active electrode of the pile is constituted by a metal capable of being attacked by the exciting-liquid of the pile when the circuit is closed—for example, zinc, tin, lead, or a metal capable of fixing the hydrogen, as palladium platinum, spongy platinum, iron reduced, or, as well, copper obtained by precipitation or electro-chemical reduction. These piles are reversible—that is to say, capable of being recharged by an electric current of sufficient electro-motive force.

In the accompanying drawings, Figure 1 shows in sectional and in plan view an apparatus adapted for practicing our invention; Fig. 2, similar views of another arrangement, and Figs. 3, 4, and 5, still other arrangements.

The following are examples of practical arrangements:

A. First. The inactive plate, Fig. 1, is formed by a plate,  $a$   $a$ , of iron, copper, or other metal, or of a plate of gas-retort carbon, surrounded

by oxide of copper,  $c$   $c$ , built up and maintained by a bag,  $c'$   $c'$   $c'$   $c'$ , of cotton or hemp cloth, or iron, copper, or brass wire-gauze. In this and the succeeding figures,  $b$  represents the negative pole,  $d$  the exciting-liquid, and  $e$  the containing-vessel. This oxide of copper can be mixed with iron filings or turnings, or copper filings or turnings, or pieces of metal gauze, or fragments of carbon to augment the surface of the depolarizing-pole.

Second. A porous vessel,  $a^2$   $a^2$   $a^2$   $a^2$ , can be employed, as shown in Fig. 2, in which is placed an iron rod,  $a'$   $a'$ , or a rod of copper, or carbon rod, surrounded with iron or copper turnings or fragments of carbon. The interstices are filled with oxide of copper.

Third. Oxide of copper is simply placed at the bottom of the vessel which forms the pile, mixed or not with conducting materials, a metallic rod, or a rod of carbon plunged in the mass and forming the positive pole. A very simple arrangement (shown in Fig. 4) consists in putting the depolarizing material  $c$  in the interior of a metal capsule or cover,  $c^2$ , placed at the bottom of the vessel  $e$ , and communicating with the exterior by an isolated conductor,  $a$ . Thus is obtained an arrangement analogous to that of Calland couples, with this difference, that the depolarizer is not soluble and that the two poles can be placed at very little distance apart.

Fourth. We are able in different ways, of which Fig. 3 illustrates one, to form with oxide of copper agglomerations or plates  $c^2$   $c^2$ , or cylinders, bricks, grains of greater or less size, which are sufficient for employment in maintaining charges near the positive pole  $a$  of the pile. Oxide of copper is equally capable of being agglomerated directly on the conductor forming the positive pole and being part of it.

(a.) Heat alone suffices to agglomerate the oxide of copper as partially melted.

(b.) This agglomeration is provided at a lower temperature on adding to the oxide of copper five to ten per cent. of pounded glass, argil, or gelatinous silica. The mixture is worked up with a sufficient quantity of water, molded, dried, and heated to a red heat.

B. For constituting the active electrode of the pile we prefer generally zinc, which gives the

greatest electro-motive force. It is useful to amalgamate it. We employ it in any form—plane surfaces, cylinders, spirals, threads, grains, bars or ingots, castings, and other forms. 5 It is applied so as to avoid all contact with the positive pole. In case the oxide is placed at the bottom of the vessel, the zinc is suspended at the upper part. To apply this arrangement to very small piles we proceed in 10 the following manner, and as shown at Fig. 5. In a cylindrical glass tube, *e*, we place a metallic wire, *a'*, having its extremity, *a<sup>3</sup>*, wound into a spiral form. We add a certain quantity of oxide of copper, *c*, which we recover in case 15 of need with porous wad, paper card, cotton, or other suitable material. We then pour in the exciting-liquid *d* and stop the mouth of the tube *e* with a stopper or cork, *f*, pierced with two orifices, *f' f<sup>2</sup>*, into one of which passes the metallic wire *a'*, while the other is traversed by a small cylinder of zinc, *b*.

20 *C. Exciting-liquid.*—As an exciting-liquid we employ solutions of caustic soda or caustic potash containing from ten to thirty per cent. 25 of the dry material.

25 *D. Working of the pile.*—A pile being constituted by a depolarizing-electrode having one of the arrangements previously described, (A,) a cylinder or a rod of zinc maintained at 30 a suitable distance, (B,) and an exciting-liquid (C) when the poles are reunited, an electric current is established in the exterior circuit. The zinc is attacked, is dissolved, or is precipitated in the state of oxide, and the oxide 35 of copper is reduced to the metallic state. The reaction is continued and the current is maintained until one of the three elements is used up—zinc, depolarizing material, or the exciting-

liquid. The pile does not work in a sensible manner while the circuit is open. When re- 40 charging the pile with a current of electricity the reduced copper absorbs oxygen energetically and returns into a state of oxide, the zinc is deposited in a metallic state, and the alkaline solution is regenerated. 45

Having fully described our invention and the means by which the same may be carried into effect, we would have it understood that we do not confine ourselves to the precise details or arrangements hereinbefore described, 50 as the same may be varied without altering the principle or the nature of our invention; but

What we desire to claim and secure by Letters Patent is—

55 1. In electric piles or galvanic batteries, oxide of copper as the depolarizing-body, combined with caustic potash or caustic soda in solution as the exciting-liquid, zinc forming the active electrode of the pile or battery, substantially as hereinbefore described.

2. In electric piles or galvanic batteries, oxide of copper and caustic soda or caustic potash in solution, in combination with the devices herein described for maintaining the oxide of 60 copper in contact with the inactive plate of the battery or pile.

FELIX DE LALANDE.  
GEORGES CHAPERON.

Witnesses as to F. de Lalande:

A. MILLOT,  
E. P. MACLEAN.

Witnesses as to G. Chaperon:

EDUARDO DIAN,  
V. DELIGNY.